

## UNITED STATES PATENT OFFICE

WILHELM HIRSCHKIND, OF ANTIOCH, CALIFORNIA, ASSIGNOR TO GREAT WESTERN ELECTRO-CHEMICAL CO., OF SAN FRANCISCO, CALIFORNIA, A CORPORATION OF CALIFORNIA

## PAPER PULP BLEACHING PROCESS

No Drawing.

Application filed December 3, 1928. Serial No. 323,575.

REISSUED

This invention relates to the bleaching of wood pulp, either ground wood or mechanical pulp, or chemical wood pulp as derived from the soda, sulphate or sulphite processes and the object of the process is to lighten the color of such pulps while preserving the strength and paper yield to the maximum.

The purpose of my process is not to produce highly bleached or white pulp but rather to cause a lightening of the original dark color. For instance, ground wood pulp can not be converted into a white pulp because all of the lignin and incrusting matters are still present, and which preclude the use of oxidizing agents as for instance chlorine so necessary for producing white pulp. The dark color of such pulp can be lightened somewhat by treatment with reducing agents, and some of these have been so used for some time.

It is also common knowledge that sulphur dioxide gas or bisulphite liquor will brighten or lighten dark pulps to some extent. The action however is slow and the quantity of sulphite necessary to use is considerable.

I have discovered that the compound, sodium hydrosulphite of the chemical composition  $Na_2S_2O_4$ , has a lightening action on the color of wood pulp infinitely greater and far more rapid than sulphur dioxide or bisulphites. I found that sodium hydrosulphite when added to very darkly colored mechanical wood pulp in a quantity of one quarter of one per cent by weight and thoroughly mixed therewith in the presence of water, produced a lightening of the color far beyond any effect obtainable with the bisulphites, and that the whole process was completed in very few minutes.

Ground wood which has been in storage for some time gradually darkens and produces a paper, after treatment in the ordinary way, which is considerably off color, whereas a hydrosulphite added to the pulp in quantities of as little as one quarter of one per cent of the weight of the dry ground wood pulp will bring back the color of fresh ground wood, and a very small additional quantity will lighten the color beyond the original color.

Kraft pulp as produced by the sulphate

process is naturally very dark in color and can be considerably improved by the use of one to two per cent of a hydrosulphite.

Even the color of sulphite pulp can be considerably lightened and improved by small quantities of a hydrosulphite, without of course reaching the color of the so called bleached sulphite pulp produced with hypochlorites.

I have already mentioned the rapidity of the action of the hydrosulphite in treatment of paper pulp and it is quite remarkable that this action is hardly influenced by temperature ranges between 50° F. and 120° F. so that at the rather low temperatures of approximately 50° F. the effect is just the same.

Sodium hydrosulphite has been mentioned above because it is the cheapest and best known representative of these compounds. But other hydrosulphites, such as potassium or ammonium hydrosulphite, calcium, or those of the alkaline earth group have been used by me with satisfactory results, and zinc hydrosulphite ( $ZnS_2O_4$ ) which is particularly easy to manufacture has also been found suitable for this purpose.

A further advantage of the use of a hydrosulphite for the bleaching of paper pulp is the ease of its application. It can be dissolved in water and run as an aqueous solution into a mixer or beater where the pulp is being mixed or it can be added as a solid direct to the wet pulp and thoroughly incorporated therewith. Since the reaction is completed within very few minutes it is only necessary to add the hydrosulphite to the beater or mixer in which the pulp is agitated before going to the paper machines.

As an example of its application to news print paper 2,300 pounds of ground wood pulp were mixed with 400 pounds of sulphite pulp to a stock density of approximately five per cent. Five and three-quarters pounds of anhydrous sodium hydrosulphite were added to this mixture. Ten minutes later the necessary sizing and bluing ingredients were added to the batch and the material was run directly on the paper machine.

News print paper resulting from a mixture

of about 83% ground wood to about 17% bleached sulphite pulp may be closely approximated in grade by using unbleached sulphite pulp with the ground wood if a small quantity of a hydrosulphite is incorporated in the proportions indicated. The advantages are in substituting the cheaper unbleached sulphite pulp for the bleached pulp ordinarily required.

10 Since various quantities of the chemical from .25% to 10% of the weight of the pulp produce corresponding degrees of action on the color of the pulp and the amount to be used will be governed entirely by the effects 15 desired, I do not confine myself to any particular quantity or percentage of the chemical to the pulp treated.

I claim:

1. The process of lightening the color of 20 mechanical wood pulp which comprises agitating the same substantially at room temperature for about ten minutes with an aqueous solution of a hydrosulphite as substantially the only active agent therein and 25 in amount ranging from .25% to 10% of the weight of the pulp without subsequent washing.

2. The process of lightening the color of 30 mechanical wood pulp which comprises agitating the same substantially at room temperature for about ten minutes with an aqueous solution of sodium hydrosulphite substantially as the only active agent therein and in amount ranging from .25% to 10% 35 of the weight of the pulp without subsequent washing.

3. The process of making paper from 40 mechanical wood pulp, which comprises agitating the pulp at substantially room temperature for a short time with an aqueous solution of a hydrosulphite as substantially the only active bleaching agent therein and in amount ranging from .25% to 10% of the weight of the pulp, and without subsequent 45 washing converting the pulp into paper before reversion of color can take place in the pulp.

WILHELM HIRSCHKIND.

50

55

60